



US009096956B2

(12) **United States Patent**  
Shiflett et al.

(10) **Patent No.:** US 9,096,956 B2  
(45) **Date of Patent:** Aug. 4, 2015

(54) **PROCESS FOR THE PRODUCTION OF CARBON FIBERS FROM POLY( $\alpha$ (1→3) GLUCAN) FIBERS**

(71) Applicant: **E I DU PONT DE NEMOURS AND COMPANY**, Wilmington, DE (US)

(72) Inventors: **Mark Brandon Shiflett**, Wilmington, DE (US); **Beth Ann Elliott**, Claymont, DE (US)

(73) Assignee: **E I DU PONT DE NEMOURS AND COMPANY**, Wilmington, DE (US)

(\*) Notice: Subject to any disclaimer, the term of this patent is extended or adjusted under 35 U.S.C. 154(b) by 389 days.

(21) Appl. No.: **13/770,068**

(22) Filed: **Feb. 19, 2013**

(65) **Prior Publication Data**

US 2013/0214443 A1 Aug. 22, 2013

**Related U.S. Application Data**

(60) Provisional application No. 61/600,338, filed on Feb. 17, 2012.

(51) **Int. Cl.**  
**D01F 9/16** (2006.01)  
**D01F 9/24** (2006.01)

(52) **U.S. Cl.**  
CPC ... **D01F 9/24** (2013.01); **D01F 9/16** (2013.01)

(58) **Field of Classification Search**  
CPC ..... D01F 9/12; D01F 9/14; D01F 9/16;  
D01F 9/20; D01F 9/24; Y10S 264/19  
USPC ..... 264/29.2, 29.6, 29.7, DIG. 19  
See application file for complete search history.

(56) **References Cited**

**U.S. PATENT DOCUMENTS**

3,552,923 A \* 1/1971 Carpenter et al. .... 423/447.6  
3,723,609 A \* 3/1973 Mansmann et al. .... 423/447.1  
4,501,886 A 2/1985 O'Brien  
7,000,000 B1 2/2006 O'Brien

**OTHER PUBLICATIONS**

Simpson, Christine L. et al., Four glucosyltransferases, GtfJ, GtfK, GtfL and GtfM, from *Streptococcus salivarius* ATCC 25975, *Microbiology*, 1995, pp. 1451-1460, vol. 141, Month of Publication Unknown.

\* cited by examiner

*Primary Examiner* — Michael Tolin

(57) **ABSTRACT**

A process is provided for preparation of carbon fibers based from fibers of poly( $\alpha$ (1→3) glucan). The method comprises three thermal exposures at progressively higher temperatures to drive off volatiles, thermally stabilize the glucan fiber, and carbonize the thermally stabilized fiber. The carbon fibers prepared according to the process hereof are strong, stiff, tough, and easily handled.

**5 Claims, 4 Drawing Sheets**







FIG. 2



FIG. 3



Front View

FIG. 4B



Top View

FIG. 4A

## 1

**PROCESS FOR THE PRODUCTION OF  
CARBON FIBERS FROM POLY( $\alpha$ (1 $\rightarrow$ 3)  
GLUCAN) FIBERS**

**FIELD OF THE INVENTION**

The invention relates to carbon fibers, processes of preparing the carbon fibers and the use of the carbon fibers in various applications.

**BACKGROUND OF THE INVENTION**

Carbon fibers are generally defined as a fiber containing at least about 92 wt-% of carbon. Carbon fibers containing 99 wt-% or more of carbon are often referred to as graphite fibers. Carbon fibers (CFs) are used in various applications owing to their excellent tensile properties, thermal and chemical stabilities (in absence of oxidizing agents) and thermal and electrical conductivities. The conventional applications of CFs include aircraft frames, turbine blades, automobile panels, sporting goods and industrial components.

Currently, the carbon fiber market is dominated by carbon fiber derived from polyacrylonitrile (PAN), with the balance being made up of fibers from pitch and rayon. CFs with distinct properties result from the processing of different precursor fibers. In a typical process in the art for converting organic polymer fibers into carbon fibers, the organic polymer fiber is first heat-stabilized in air in an oxidation process conducted at a temperature of 200 to 400° C. The thus stabilized precursor fibers then undergo controlled pyrolysis, i.e., a carbonization step, comprising heat-treating in an inert atmosphere such as nitrogen to a temperature of from about 300° C. to about 3000° C., which removes non-carbon elements such as hydrogen, oxygen and nitrogen from the oxidized fiber. It is known in the art that heating at the higher end of the temperature spectrum, e.g., between about 1000° C. and about 3000° C. may achieve higher carbon content, thereby producing CFs with higher Young's modulus values.

For automotive applications, desired mechanical properties for carbon fibers include tensile strength of >1.72 GPa, tensile modulus of >172 GPa and elongation at break of about 1%.

In addition to the limited mechanical properties of conventional CFs, the currently used methods of preparing CFs can be costly. For example, the cost of the precursor fiber amounts to approximately 40% to 50% of the total cost of preparing the carbon fiber. Therefore, there is a need in the art for lower cost precursor fibers that yield carbon fibers of excellent quality would significantly reduce the cost of CFs. An additional benefit would be to enable the expansion of CF applications to industries and markets such as those related to the automotive industry.

Furthermore, it is desirable to provide a source of carbon fibers that derives from a renewable source that does not contribute to global warming.

Polysaccharides have been known since the dawn of civilization, primarily in the form of cellulose, a polymer formed from glucose by natural processes via  $\beta$ (1 $\rightarrow$ 4) glycoside linkages; see, for example, *Applied Fibre Science*, F. Happey, Ed., Chapter 8, E. Atkins, Academic Press, New York, 1979. Numerous other polysaccharide polymers are also disclosed therein.

Only cellulose among the many known polysaccharides has achieved commercial prominence as a fiber. In particular, cotton, a highly pure form of naturally occurring cellulose, is well-known for its beneficial attributes in textile applications.

It is further known that cellulose exhibits sufficient chain extension and backbone rigidity in solution to form liquid crystalline solutions; see, for example O'Brien, U.S. Pat. No. 4,501,886. The teachings of the art suggest that sufficient

## 2

polysaccharide chain extension could be achieved only in  $\beta$ (1 $\rightarrow$ 4) linked polysaccharides and that any significant deviation from that backbone geometry would lower the molecular aspect ratio below that required for the formation of an ordered phase.

More recently, glucan polymer, characterized by  $\alpha$ (1 $\rightarrow$ 3) glycoside linkages, has been isolated by contacting an aqueous solution of sucrose with GtfJ glucosyltransferase isolated from *Streptococcus salivarius*, Simpson et al., *Microbiology*, vol 141, pp. 1451-1460 (1995). Highly crystalline, highly oriented, low molecular weight films of  $\alpha$ (1 $\rightarrow$ 3)-D-glucan have been fabricated for the purposes of x-ray diffraction analysis, Ogawa et al., *Fiber Diffraction Methods*, 47, pp. 353-362 (1980). In Ogawa, the insoluble glucan polymer is acetylated, the acetylated glucan dissolved to form a 5% solution in chloroform and the solution cast into a film. The film is then subjected to stretching in glycerine at 150° C. which orients the film and stretches it to a length 6.5 times the original length of the solution cast film. After stretching, the film is deacetylated and crystallized by annealing in superheated water at 140° C. in a pressure vessel. It is well-known in the art that exposure of polysaccharides to such a hot aqueous environment results in chain cleavage and loss of molecular weight, with concomitant degradation of mechanical properties.

Polysaccharides based on glucose and glucose itself are particularly important because of their prominent role in photosynthesis and metabolic processes. Cellulose and starch, both based on molecular chains of polyanhydroglucosamine are the most abundant polymers on earth and are of great commercial importance. Such polymers offer materials that are environmentally benign throughout their entire life cycle and are constructed from renewable energy and raw materials sources.

The term "glucan" is a term of art that refers to a polysaccharide comprising beta-D-glucose monomer units that are linked in eight possible ways. Cellulose is a glucan.

Within a glucan polymer, the repeating monomeric units can be linked in a variety of configurations following an enchainment pattern. The nature of the enchainment pattern depends, in part, on how the ring closes when an aldohexose ring closes to form a hemiacetal. The open chain form of glucose (an aldohexose) has four asymmetric centers (see below). Hence there are 2<sup>4</sup> or 16 possible open chain forms of which D and L glucose are two. When the ring is closed, a new asymmetric center is created at C1 thus making 5 asymmetric carbons. Depending on how the ring closes, for glucose,  $\alpha$ (1 $\rightarrow$ 4)-linked polymer, e.g. starch, or  $\beta$ (1 $\rightarrow$ 4)-linked polymer, e.g. cellulose, can be formed upon further condensation to polymer. The configuration at C1 in the polymer determines whether it is an alpha or beta linked polymer, and the numbers in parenthesis following alpha or beta refer to the carbon atoms through which enchainment takes place.





\* asymmetric carbon center

The properties exhibited by a glucan polymer are determined by the enchainment pattern. For example, the very different properties of cellulose and starch are determined by the respective nature of their enchainment patterns. Starch or amylose consists of  $\alpha(1\rightarrow 4)$  linked glucose and does not form fibers among other things because it is swollen or dissolved by water. On the other hand, cellulose consists of  $\beta(1\rightarrow 4)$  linked glucose, and makes an excellent structural material being both crystalline and hydrophobic, and is commonly used for textile applications as cotton fiber, as well as for structures in the form of wood.

Like other natural fibers, cotton has evolved under constraints wherein the polysaccharide structure and physical properties have not been optimized for textile uses. In particular, cotton fiber is of short fiber length, limited variation in cross section and fiber fineness and is produced in a highly labor and land intensive process.

O'Brien, U.S. Pat. No. 7,000,000 discloses a process for preparing fiber from liquid crystalline solutions of acetylated poly( $\alpha(1\rightarrow 3)$  glucan). The thus prepared fiber was then deacetylated resulting in a fiber of poly( $\alpha(1\rightarrow 3)$  glucan).

The inventive method described herein, results in carbon fibers meeting these desired mechanical benchmarks and would further reduce the costs making CFs available to additional industrial sectors.

#### SUMMARY OF THE INVENTION

A process comprising subjecting one or more filaments of poly( $\alpha(1\rightarrow 3)$  glucan) to a tension below the breaking strength of the one or more filaments at 350° C.; subjecting the thus tensioned one or more filaments to a first thermal exposure by heating said one or more filaments to a temperature in the range of 160 to 200° C. in air for a duration in the range of 5 to 15 minutes; subjecting the thus heated one or more filaments to a second thermal exposure by further heating said one or more filaments at a heating rate, still under tension, from a first temperature in the range of 200 to 250° C. to a second temperature in the range of 300 to 350° C., said heating rate being in the range of 0.1 to 1° C. per minute, thereby preparing one or more thermally stabilized filaments; subjecting said one or more stabilized filaments in a zero tension state to a third thermal exposure by heating said one or stabilized filaments to a temperature in the range of 700 to 1500° C. in an inert atmosphere for a duration in the range of 0.5 to 5 minutes, thereby preparing one or more carbonized filaments.

#### BRIEF DESCRIPTION OF THE DRAWINGS

FIG. 1 depicts a side view of the fiber spinning apparatus employed in the specific embodiments hereof.

FIG. 2 depicts a side view of the tube furnace arrangement used in the thermal stabilization step of the process hereof as executed in the specific embodiments thereof.

FIG. 3 depicts a side view of the carbonization apparatus used in the specific embodiments hereof.

FIG. 4A depicts a top view, and FIG. 4B depicts a front view of the winding frame used to prepare the filament skeins employed in the specific embodiments hereof.

#### 10 DETAILED DESCRIPTION OF THE INVENTION

When a range of values is provided herein, it is intended to encompass the end-points of the range unless specifically stated otherwise. Numerical values used herein have the precision of the number of significant figures provided, following the standard protocol in chemistry for significant figures as outlined in ASTM E29-08 Section 6. For example, the number 40 encompasses a range from 35.0 to 44.9, whereas the number 40.0 encompasses a range from 39.50 to 40.49.

20 As used herein, the term "filament" encompasses a thread-shaped compact unit comprising one or more molecules of a polymer comprising poly( $\alpha(1\rightarrow 3)$  glucan). The filament can further comprise additional polymers added, for example, order to control the morphology of the carbon fiber produced according to the process hereof. Such additives as are commonly employed in the art of carbon fiber production to enhance the properties or processing of organic polymers undergoing solution spinning and subsequent carbonization can also be included.

25 In the present invention, the term "fiber" and the term "filament" are used interchangeably. The present invention is directed to the preparation of high strength, high modulus carbon fibers from a fiber precursor comprising poly( $\alpha(1\rightarrow 3)$  glucan). Suitable poly( $\alpha(1\rightarrow 3)$  glucan) fibers are in the form of continuous filaments. Staple fibers are not well suited for the practice of the present invention.

30 According to the present invention a process is provided for the preparation of carbon fiber from a precursor fiber comprising poly( $\alpha(1\rightarrow 3)$  glucan), the process comprising subjecting one or more filaments comprising poly( $\alpha(1\rightarrow 3)$

35 glucan) to a tension below the breaking strength of the one or more filaments at 350° C.;

subjecting the thus tensioned one or more filaments to a first thermal exposure by heating said one or more filaments to a temperature in the range of 160 to 200° C. in air for a duration in the range of 5 to 15 minutes;

subjecting the thus heated one or more filaments to a second thermal exposure by further heating said one or more filaments at a heating rate, still under tension, from a first temperature in the range of 200 to 250° C. to a second temperature in the range of 300 to 350° C., said heating rate being in the range of 0.1 to 1° C. per minute, thereby preparing one or more thermally stabilized filaments;

subjecting said one or more stabilized filaments in a zero tension state to a third thermal exposure by heating said one or stabilized filaments to a temperature in the range of 700 to 1500° C. in an inert atmosphere for a duration in the range of 0.5 to 5 minutes, thereby preparing one or more carbonized filaments.

One benefit of the present invention over the known art is that the carbon fiber resulting from the process hereof is a "green" product—that is, it is biologically sourced because the poly( $\alpha(1\rightarrow 3)$  glucan) upon which it is based is produced by fermentation, and not from petroleum.

60 If the first thermal exposure is conducted at a temperature below 160° C., it may be ineffective. If the first thermal

exposure is conducted at a temperature above 200° C., it can cause water molecules trapped within fiber pores to evaporate too quickly and rupture the fiber, causing points of weakness where the fiber can break. The duration of exposure less than 5 minutes is not highly effective. An exposure of greater than 15 minutes is not deleterious, but is unnecessary. In one embodiment of the process hereof, the first thermal exposure is effected at a temperature in the range of 175 to 185° C. for a duration of 7.5 to 12.5 minutes.

Thermal stabilization of the poly( $\alpha$ (1 $\rightarrow$ 3) glucan) fiber is effected in a second thermal exposure, which involves heating from a first temperature in the range 200 to 250° C., preferably 230 to 250° C., to a second temperature in the range of 300 to 350° C., preferably 310 to 330° C. At a temperature below 200° C., thermal stabilization does not occur or occurs at a rate that is impractically slow. At a temperature above 350° C., the fiber can melt and break.

In one embodiment of the process hereof, said second thermal exposure is effected in a series of well-defined steps between the first temperature and the second temperature, with a hold period between steps, and a heating rate from step to step in excess of 10° C. per minute.

The first and second thermal exposures are conducted in air or an oxygen containing atmosphere. If the first and second thermal exposures are conducted in an oxygen containing atmosphere other than air, the same sequence of steps will still be operative, but will be modified in detail to accommodate the atmosphere in question.

The third thermal exposure, the carbonization step, is effected in an inert environment. Any inert environment is satisfactory. A heavy nitrogen purge, as described in the specific embodiments infra, has been found to be satisfactory. The third thermal exposure is conducted in the temperature range of 700 to 1500° C., preferably 800 to 1000° C. At a temperature below 700° C., the necessary level of pyrolysis and carbonization does not occur. At temperatures above 1500° C., the resulting carbon fiber can undergo such deleterious changes as loss of integrity, melting and others.

When the third thermal exposure is conducted for a period of time less than 0.5 minutes, insufficient carbonization takes place. For a period of time more than 5 minutes, the resulting carbon fiber may undergo deleterious changes, particularly in the higher range of carbonization temperatures. In one embodiment, the third thermal exposure is effected in the temperature range of 800 to 1000° C. for a period of time of 1 to 2 minutes.

The resulting carbon fiber is strong, very stiff, and tough.

The invention is further described in, but not limited by, the following specific embodiments.

## Examples

## Materials

| MATERIAL        | Description                                          | Vendor                               |
|-----------------|------------------------------------------------------|--------------------------------------|
| Dialysis tubing | Spectrapor 25225-226, 12000 molecular weight cut-off | VWR (Radnor, PA).                    |
| Sucrose         | 15 wt-% solids aqueous solution (#BDH8029)           | VWR.                                 |
| Dextran         | T-10 (#D9260)                                        | Sigma Aldrich.                       |
| Ethanol         | Undenatured (#459844)                                | Sigma Aldrich                        |
| Antifoam        | Suppressor 7153                                      | Cognis Corporation (Cincinnati, OH). |

All other chemicals were obtained from commonly used suppliers of such chemicals.

## Preparation of Glucosyltransferase (gtfJ) Enzyme Seed Medium

- 5 The seed medium, used to grow the starter cultures for the fermenters, contained: yeast extract (Amberex 695, 5.0 grams per liter, g/L), K<sub>2</sub>HPO<sub>4</sub> (10.0 g/L), KH<sub>2</sub>PO<sub>4</sub> (7.0 g/L), sodium citrate dihydrate (1.0 g/L), (NH<sub>4</sub>)<sub>2</sub>SO<sub>4</sub> (4.0 g/L), MgSO<sub>4</sub> heptahydrate (1.0 g/L) and ferric ammonium citrate (0.10 g/L).
- 10 The pH of the medium was adjusted to 6.8 using either 5N NaOH or H<sub>2</sub>SO<sub>4</sub> and the medium was sterilized in the flask. Post sterilization additions included glucose (20 mL/L of a 50% w/w solution) and ampicillin (4 mL/L of a 25 mg/mL stock solution).

## 15 Fermenter Medium

- The growth medium used in the fermenter contained: KH<sub>2</sub>PO<sub>4</sub> (3.50 g/L), FeSO<sub>4</sub> heptahydrate (0.05 g/L), MgSO<sub>4</sub> heptahydrate (2.0 g/L), sodium citrate dihydrate (1.90 g/L), yeast extract (Amberex 695, 5.0 g/L), Suppressor 7153 anti-foam (0.25 milliliters per liter, mL/L), NaCl (1.0 g/L), CaCl<sub>2</sub> dihydrate (10 g/L), and NIT trace elements solution (10 mL/L). The NIT trace elements solution contained citric acid monohydrate (10 g/L), MnSO<sub>4</sub> hydrate (2 g/L), NaCl (2 g/L), FeSO<sub>4</sub> heptahydrate (0.5 g/L), ZnSO<sub>4</sub> heptahydrate (0.2 g/L), CuSO<sub>4</sub> pentahydrate (0.02 g/L) and NaMoO<sub>4</sub> dihydrate (0.02 g/L). Post sterilization additions included glucose (12.5 g/L of a 50% w/w solution) and ampicillin (4 mL/L of a 25 mg/mL stock solution).

## 20 Construction of Glucosyltransferase (gtfJ) Enzyme Expression Strain

- 25 A gene encoding the mature glucosyltransferase enzyme (gtfJ; EC 2.4.1.5; GENBANK® AAA26896.1, SEQ ID NO: 3) from *Streptococcus salivarius* (ATCC 25975) was synthesized using codons optimized for expression in *E. coli* (DNA 3.0, Menlo Park Calif.). The nucleic acid product (SEQ ID NO: 1) was subcloned into pJexpress404® (DNA 2.0, Menlo Park Calif.) to generate the plasmid identified as pMP52 (SEQ ID NO: 2). The plasmid pMP52 was used to transform *E. coli* MG1655 (ATCC47076™) to generate the strain identified as MG1655/pMP52. All procedures used for construction of the glucosyltransferase enzyme expression strain are well known in the art and can be performed by individuals skilled in the relevant art without undue experimentation.

## 30 Production of Recombinant gtfJ in Fermentation

- 35 Production of the recombinant gtfJ enzyme in a fermenter was initiated by preparing a pre-seed culture of the *E. coli* strain MG1655/pMP52, expressing the gtfJ enzyme, constructed as described infra. A 10 mL aliquot of the seed medium was added into a 125 mL disposable baffled flask and 50 was inoculated with a 1.0 mL culture of *E. coli* MG1655/pMP52 in 20% glycerol. This culture was allowed to grow at 37° C. while shaking at 300 revolutions per minute (rpm) for 3 hours.

- 40 A seed culture, for starting the fermenter, was prepared by 55 charging a 2 L shake flask with 0.5 L of the seed medium. 1.0 mL of the pre-seed culture was aseptically transferred into 0.5 L seed medium in the flask and cultivated at 37° C. and 300 rpm for 5 hours. The seed culture was transferred at optical density 550 nm (OD<sub>550</sub>)>2 to a 14 L fermenter (Braun, Perth Amboy, N.J.) containing 8 L of the fermenter medium described above at 37° C.

- 60 Cells of *E. coli* MG1655/pMP52 were allowed to grow in the fermenter and glucose feed (50% w/w glucose solution containing 1% w/w MgSO<sub>4</sub>·7H<sub>2</sub>O) was initiated when glucose concentration in the medium decreased to 0.5 g/L. The feed was started at 0.36 grams feed per minute (g feed/min) and increased progressively each hour to 0.42, 0.49, 0.57,

0.66, 0.77, 0.90, 1.04, 1.21, 1.41, 1.63, 1.92, 2.2 g feed/min respectively. The rate was held constant afterwards by decreasing or temporarily stopping the glucose feed when glucose concentration exceeded 0.1 g/L. Glucose concentration in the medium was monitored using a YSI glucose analyzer (YSI, Yellow Springs, Ohio).

Induction of glucosyltransferase enzyme activity was initiated, when cells reached an  $OD_{550}$  of 70, with the addition of 9 mL of 0.5 M IPTG (isopropyl  $\beta$ -D-1-thiogalacto-pyranoside). The dissolved oxygen (DO) concentration was controlled at 25% of air saturation. The DO was controlled first by impeller agitation rate (400 to 1200 rpm) and later by aeration rate (2 to 10 standard liters per minute, slpm). The pH was controlled at 6.8.  $NH_4OH$  (14.5% weight/volume, w/v) and  $H_2SO_4$  (20% w/v) were used for pH control. The back pressure was maintained at 0.5 bars. At various intervals (20, 25 and 30 hours), 5 mL of Suppressor 7153 antifoam was added into the fermenter to suppress foaming. Cells were harvested by centrifugation 8 hours post IPTG addition and were stored at  $-80^\circ C$ . as a cell paste.

#### Preparation of gtfJ Crude Enzyme Extract from Cell Paste

The cell paste obtained above was suspended at 150 g/L in 50 mM potassium phosphate buffer pH 7.2 to prepare a slurry. The slurry was homogenized at 12,000 psi (Rannie-type machine, APV-1000 or APV 16.56) and the homogenate chilled to  $4^\circ C$ . With moderately vigorous stirring, 50 g of a floc solution (Aldrich no. 409138, 5% in 50 mM sodium phosphate buffer pH 7.0) was added per liter of cell homogenate. Agitation was reduced to light stirring for 15 minutes. The cell homogenate was then clarified by centrifugation at 4500 rpm for 3 hours at 5-10° C. Supernatant, containing crude gtfJ enzyme extract, was concentrated (approximately 5 $\times$ ) with a 30 kilo Dalton (kDa) cut-off membrane. The concentration of protein in the gtfJ enzyme solution was determined by the bicinchoninic acid (BCA) protein assay (Sigma Aldrich) to be 4.8 g/L.

#### Enzymatic Synthesis of Poly( $\alpha$ (1 $\rightarrow$ 3) Glucan)

Several batches of poly( $\alpha$ (1 $\rightarrow$ 3) glucan) polymer were prepared by combining the materials listed in Table 1 in the amounts shown. The pH was adjusted to pH 6.8-7.0 by addition of 10% KOH. De-ionized water was then added to bring the volume up to level specified in Table 1. The buffer concentration in the thus prepared solution was 50 mM.

The thus prepared pH-adjusted solution was then charged with the enzyme extract prepared supra in an amount sufficient to bring the enzyme concentration to 0.30% by weight in each batch. Each thus prepared reaction mixture was then allowed to stand at ambient temperature for 144 hours. The resulting poly( $\alpha$ (1 $\rightarrow$ 3) glucan) solids were collected on a Buchner funnel using a 325 mesh screen over 40 micron filter paper. The filter cake was re-suspended in deionized water and filtered twice more as above to remove sucrose, fructose and other low molecular weight, soluble by-products. Finally two additional washes with methanol were carried out, the filter cake was pressed out thoroughly on the funnel and dried in vacuum at room temperature, yielding a white flaky solid in the amounts shown in Table 1.

TABLE 1

| Batch Number | Batch size (L) | Sucrose (g) | Dextran T-10 (g) | KH <sub>2</sub> PO <sub>4</sub> Buffer (mL) | Ethanol (mL) | Yield |
|--------------|----------------|-------------|------------------|---------------------------------------------|--------------|-------|
| 1            | 20             | 1000        | 4.0              | 1000                                        | 0            | 120.0 |
| 2            | 20             | 1000        | 4.0              | 1000                                        | 0            | 114.5 |
| 3            | 20             | 1000        | 4.0              | 1000                                        | 0            | 113.0 |

TABLE 1-continued

| Batch Number | Batch size (L) | Sucrose (g) | Dextran T-10 (g) | KH <sub>2</sub> PO <sub>4</sub> Buffer (mL) | Ethanol (mL) | Yield |
|--------------|----------------|-------------|------------------|---------------------------------------------|--------------|-------|
| 4            | 20             | 1000        | 4.0              | 1000                                        | 0            | 86.0  |
| 5            | 3              | 450         | 2.4              | 150                                         | 150          | 47.3  |
| 6            | 3              | 450         | 3.0              | 150                                         | 300          | 32.1  |
| 7            | 3              | 450         | 6.0              | 150                                         | 300          | 49.0  |
| 8            | 3              | 450         | 9.0              | 150                                         | 300          | 56.6  |

#### Preparation of 1,3 Alpha Glucan Triacetate

The several batches of poly( $\alpha$ (1 $\rightarrow$ 3) glucan) as shown in Table 1 were combined in the amounts shown, respectively, in Table 2 to make three 130 g blends for subsequent acetylation.

The blends were boiled for one hour in deionized water. Each thus boiled blend was then added to a mixture containing 890 mL of methylene chloride, 600 mL of acetic acid and 870 mL of acetic anhydride in a 4 L reaction kettle provided with a nitrogen blanket. Mixing was effected with an egg beater style mixing blade that covered the entire depth of the liquid. The resulting mixture was then cooled to approximately  $-5^\circ C$ . Separately, a catalyst mixture was prepared by addition of 9 mL of 70% aqueous perchloric acid to 370 mL of chilled acetic anhydride. The catalyst mixture was then added dropwise to the rapidly stirred reaction mixture at  $-5^\circ C$ . Subsequent to catalyst addition, the reaction kettle was immersed in a hot water bath contained in a 2 gallon plastic bucket, and heated to  $30^\circ C$ . When the temperature of the reactants was observed to exceed  $32^\circ C$ ., the reaction kettle was removed from the hot water bath and suspended in the air until the reaction temperature was observed to reach  $27^\circ C$ . at which point the reaction kettle was again immersed in the hot water bath. This procedure was continued for a period of 2-4 hours until reaction was complete. The reaction was deemed to be complete when no particulate matter was observed by visual inspection of the translucent reaction mixture.

In small aliquots, the mixture was coagulated in methanol in a Waring blender, the resultant suspension was filtered, washed with methanol twice more, water washed until neutral pH was obtained, and then washed with methanol and dried under vacuum. Yield of the resulting triacetate is shown in Table 2

TABLE 2

| Blend | Polymer Batches | Wt. (g)     | Triacetate Yield (g) |
|-------|-----------------|-------------|----------------------|
| 1     | 1/2             | 30/100      | 190.4                |
| 2     | 3/4             | 43.7/86.3   | 204.6                |
| 3     | 5/6/7/8         | 25/20/40/45 | 207.94               |

#### Spinning Solution

Spinning solutions A and B were prepared from the thus prepared acetylated poly( $\alpha$ (1 $\rightarrow$ 3) glucan). 100 parts by weight of trifluoroacetic acid were diluted with 8 parts by weight of water. The thus prepared solution was added to two 1-quart zip-lock bags, each containing 120 g of the respective acetylate poly( $\alpha$ (1 $\rightarrow$ 3) glucan) blends, as indicated in Table 3, in an amount sufficient to prepare a 37.5% solids solution in each case. Each bag was then sealed, and was subject to hand kneading to homogenize. The bag was allowed to stand at ambient conditions overnight. In order to dissolve the polymer therein, the mixture of polymer and solvent was first stirred by hand using a stainless steel spatula in order to homogenize the mixture. The homogenized mixture was then

pumped back and forth through 13 cycles between two syringes connected by a short length of 3 mm ID stainless steel tubing.

TABLE 3

| Spinning | Glucan Triacetate Blend |            |
|----------|-------------------------|------------|
| Solution | #                       | Weight (g) |
| A        | 1                       | 94         |
|          | 2                       | 26         |
| B        | 3                       | 120        |

#### Fiber Spinning of Glucan Triacetate

The thus prepared spinning solutions were solution-spun into continuous filaments using the spinning apparatus depicted in FIG. 1. The spinning solution was charged to the cell (13) that was provided with a piston (11) connected to ram (12) which pushed solution through a spin pack containing a screen pack (14) provided with stainless steel support screens including 100 mesh support screen and a 325 mesh filter screen, and a 20-hole spinneret (15). Each spinneret hole was characterized by a diameter of 0.005 in. and a length to diameter ratio of 6. The piston (11) was driven by a drive screw (not shown) that drove the ram at a metered rate. The filaments (16) emerging from the spinneret (15) were directed into a coagulation bath (17) consisting of 100% methanol. The fiber was passed around Teflon guide pins (18) within the coagulation bath and exiting the bath to a traverse (19) with a guide pin (110) distributing the fiber evenly across a width to a windup (111) where the fiber is collected on a bobbin. The bobbins so prepared were soaked overnight in methanol. Spinning conditions are provided in Table 4. The yarns so produced are herein designated GYA-1 and GYA-2.

TABLE 4

| Spinning Solution | Jet Velocity (fpm) | Bath Temp (°C.) | Bath length (ft) | Air Gap (in) | Wind up speed (fpm) | Spin Stretch Factor |
|-------------------|--------------------|-----------------|------------------|--------------|---------------------|---------------------|
| GYA-1             | A                  | 17              | -1               | 11.8         | 0.3                 | 52                  |
| GYA-2             | B                  | 22              | -19              | 11.8         | 0.75                | 60                  |

#### Saponification

0.54 g of sodium methoxide were added to 100 mL of methanol. The bobbin of GYA-2 yarn was placed into the solution so formed for a period of 48 hours to regenerate glucan fiber from the glucan triacetate fiber. The so-treated bobbin was then rinsed with methanol, and soaked for an additional 24 hours in neat methanol, and allowed to air dry. The resulting regenerated glucan fiber yarn is herein designated GY-1.

#### Oxidation Treatment

Referring to FIG. 2, a tube furnace (21) having an entry port (22) and an exit port (22') was equipped with an air supply fan (23) that flowed air, at rates stated in Table 5, infra, into the entry port (22) and through the furnace to the exit port (22'). A skein of fiber (24) was fed end-wise through the tube furnace. The skein was disposed to pass over a pulley (25) at each end of the tube furnace. Each end of the skein was formed into a loop (26), through which a hook (27) was passed. Affixed to the hook was a weight (28). The weight employed is stated in the examples, infra. The heated section of the tube inside the tube furnace was a 2 inch schedule 5 tube with an inner diameter of 57 mm and a length of 54 inches. Each specimen was subject to a temperature of 180° C. in air

for 10 minutes. The temperature was then increased in a series of steps, as described in the thermal profile provided in the examples, infra. It took less than 1 minute to make the temperature changes between adjacent steps in the thermal profile.

#### Carbonization Treatment

Referring to FIG. 3, nitrogen was provided to the tube furnace (21) at six locations (33): one at the entry port (22) and one at the exit port (22') of the tube furnace, two at the tubing before the entrance port and two at the tubing before the exit port (22'). The nitrogen was fed through six flow meters (34). The oxidized fiber skein (35) was attached to an Inconel® transport wire 0.9 mm in diameter (36) using metal crimps (37) in order to keep the fiber skein in a zero tension state. The Inconel® wire was wrapped around pulleys (25) located at the entry port (22) and exit port (22') in order to move the fiber skein into and out of the furnace. The fiber skein thus disposed was then subject to heating according to the schedule disclosed in the specific embodiments infra.

#### Preparation of Filament Skeins.

Referring to FIG. 4, a skein of filaments having more than 20 ends was prepared by winding the skein around four posts (41) that were set at the corners of a square (42), 24 inches apart from each other. A fiber skein was wrapped around the posts until the skein contained the desired number of filaments. The skein was cut at one post, resulting in a length of 8 feet.

#### Example 1

Two 60-inch skeins, consisting each of 20 filaments of GY-1 were prepared for oxidation as described supra. To each skein, herein designated GY-1-A and GY-1-B, a 3.5-gram weight was affixed at each end as shown in FIG. 2. Under an air flow rate of 6 standard cubic feet per minute (scfm), each skein was individually heated to 230° C., held for 60 minutes, then heated to 250° C., held for 60 minutes, then heated to 270° C., held for 60 minutes, then heated to 290° C., held for 60 minutes, then heated to 310° C., held for 60 minutes. No breakage had occurred at the end of the five-hour thermal exposure process. The resulting oxidized skeins are herein designated GY-1-AO and GY-1-BO.

The GY-1-AO oxidized skein was prepared for carbonization as described supra. The skein was heated at 800° C. for 90 seconds under a nitrogen purge of 120 scfh. The skein, herein designated GY-1-AC, was removed from the oven and spooled. The skein was black in color, pliable enough to be spooled, but fragile. If the skein was wrapped tightly, filaments would break.

The GY-1-BO oxidized skein was prepared for carbonization as described supra. The skein was heated to 1000° C. for 90 seconds under a nitrogen purge of 120 scfh. The skein was black in color. The filaments seemed stronger than GY-1-AC, but upon removal from the oven, many filaments were caught on the equipment and broken.

#### Example 2

Referring to FIG. 4, a 440 filament skein was prepared by wrapping a 20-filament length of GY-1 around the posts 22 times. A second skein was prepared in the same manner. The skeins so prepared were cut at one post, resulting in two lengths of 8 feet each, designated GY-1-C and GY-1-D.

Each of GY-1-C and GY-1-D were prepared for oxidation as described, supra. Each was oxidized separately. To each skein a 50-gram weight was affixed at each end as shown in FIG. 2. Under an air flow rate of 10 scfm, each skein was

## 11

heated to 250° C., held for 40 minutes, then heated to 270° C., held for 40 minutes, then heated to 290° C., held for 40 minutes, then heated to 310° C., held for 40 minutes, then heated to 330° C., held for 40 minutes. No breakage occurred at the end of the 200-minute temperature profile. The resulting oxidized skeins are herein designated GY-1-CO and GY-1-DO.

## c. Carbonization

Oxidized skein GY-1-CO was prepared for carbonization as described supra. The skein was heated to 800° C. under a nitrogen flow rate of 120 standard scfh for 120 seconds. The thus heated skein, herein designed GY-1-CC, was removed from the furnace. The skein was black in color, pliable, and easy to spool.

Oxidized skein GY-1-DO was treated in a manner identical to that of GY-1-CO except that the temperature was 1000° C. The thus heated skein, herein designed GY-1-DC, was removed from the furnace. The skein was black in color, very pliable, and very easy to spool.

In the thus carbonized skeins fiber diameter was determined by scanning electron microscopy; denier, using a Tex-Techno Vibromat ME denier testerand (TexTechno H. Stein GMBH & Co.); and, mechanical properties, using an Instron® Universal Testing Machine. Results are shown in Table 5.

TABLE 5

|                        | GY-1-CC       | GY-1-CD       |
|------------------------|---------------|---------------|
| Diameter (micrometers) | 17.0 ± 0.4    | 19.6 ± 1.7    |
| Denier                 | 3.581 ± 0.789 | 3.076 ± 0.674 |
| Tenacity (gpd)         | 1.3 ± 0.5     | 2.0 ± 1.0     |
| Tensile Strength (MPa) | 189 ± 79      | 203 ± 100     |
| Tensile Modulus (GPa)  | 28 ± 4        | 27 ± 6        |

## Comparative Example A

One 60-inch skein consisting of 20 filaments of glucan triacetate GYA-1 was prepared for oxidation as described supra. A 4.5 g weight was affixed to each end of the skein as shown in FIG. 2. Under an air flow rate of 6 scfm, the bundle was heated to 230° C. After one minute, the skein broke.

## Comparative Example B

Two 200 filament skeins were prepared by wrapping the 20-filament glucan triacetate GYA-1 ten times around the

## SEQUENCE LISTING

<160> NUMBER OF SEQ ID NOS: 3

<210> SEQ ID NO 1  
<211> LENGTH: 4434  
<212> TYPE: DNA  
<213> ORGANISM: artificial sequence  
<220> FEATURE:  
<223> OTHER INFORMATION: codon-optimized gtfj gene from *Streptococcus salivarius*

<400> SEQUENCE: 1

|                                                                   |     |
|-------------------------------------------------------------------|-----|
| atggacgaaa cgcaggataa gaccgtgacg cagagcaaca gcgccaccac cgcttccctg | 60  |
| gtcactagcc ctgaagccac gaaagaggcg gacaaacgca cgaacactaa agaggccgac | 120 |
| gttctgacgc ctgaaaaaga aacgaacgca gtcgagactg cgaccaccac taacacccag | 180 |
| gcgacggcg aggccgccac gaccgggacc accggggacg tcgggtggc tgcgggtccg   | 240 |

## 12

posts of the apparatus in FIG. 4. Each skein was cut at one post, resulting in two lengths of 8 feet.

A 60-inch skein was cut from each of the thus prepared 8 foot lengths, herein designated GYA-1-1 and GYA-1-2. Each 60-inch skein was prepared for oxidation as described supra. Each skein was oxidized separately. A 16 g weight was affixed to each end of the GYA-1-1 skein, and a 40 g weight was affixed to each end of GYA-1-2. The skeins were heated for 10 minutes at 180° C. under an air flow rate of 6 scfm. skeins broke after 10 minutes at 180° C.

## Comparative Example C

PANOX® Thermally Stabilized Textile Fiber, an oxidized poly(acrylonitrile) fiber was obtained from The SGL Group, Ross-Shire, UK. Three PANOX fiber skeins, herein designated PANOX-1, PANOX-2, and PANOX-3, consisting of approximately 12,000 filaments per skein were prepared for carbonization as described supra. Three 60-inch length skeins were heated to 800° C. under a nitrogen atmosphere of 120 scfh. PANOX-1 was held for 60 seconds, PANOX-2 was held for 90 seconds, PANOX-3 was held for 120 seconds. PANOX-1 caught on the furnace during removal and was bunched up. No further testing was performed. PANOX-2 was frayed and could not be spooled. PANOX-3 was removed from the oven, herein designed PANOXC-3, and spooled.

A further 12,000 filament 60 inch skein of PANOX, herein designated PANOX-4, was heated to 1000° C. under a nitrogen atmosphere of 120 scfh for 120 seconds. PANOX-4 was removed from the oven, herein designated PANOXC-4 and spooled.

PANOXC-3 and PANOXC-4 were analyzed in the manner of the specimens in Example 2. Results are shown in Table 6.

TABLE 6

|                        | PANOXC-3      | PANOXC-4      |
|------------------------|---------------|---------------|
| Diameter (micrometers) | 8.0 ± 0.3     | 9.9 ± 0.3     |
| Denier                 | 0.779 ± 0.040 | 1.111 ± 0.070 |
| Tenacity (gpd)         | 9.4 ± 2.1     | 2.7 ± 1.7     |
| Tensile Strength (MPa) | 1440 ± 317    | 387 ± 247     |
| Tensile Modulus (GPa)  | 85 ± 6        | 15 ± 8        |

-continued

---

|             |             |             |             |             |             |      |
|-------------|-------------|-------------|-------------|-------------|-------------|------|
| aacaaaagaag | cggteggtac  | cacggatgt   | ccggcggtca  | cgaccgagaa  | agcggaaagaa | 300  |
| cagccggcta  | ccgttaaagc  | agaagtgcgc  | aatacggaa   | tgaaagcgcc  | ggaagcggt   | 360  |
| ctgaaaagaca | gcgagggtga  | ggcagcgctg  | agcctgaaga  | acatcaagaa  | cattgtatggc | 420  |
| aagtattact  | atgttaatga  | ggatggcagc  | cacaaagaga  | atttcgctat  | taccgtgaat  | 480  |
| ggccagctgc  | tgtactttgg  | taaagacggt  | gegctgacgt  | cctctgacac  | gtattcttt   | 540  |
| accccaggca  | ctaccaatat  | cgtggacggt  | tttagcatta  | acaaccgcgc  | ttacgacagc  | 600  |
| agcgaggcga  | gctttgagct  | gategacggt  | tacttgaccg  | cagacagctg  | gtatcgccg   | 660  |
| gctagcatca  | tcaaagatgg  | tgttacgtgg  | caagcgtcca  | ccgcccggaa  | ttttcgccg   | 720  |
| ctgctgatgg  | catggtggcc  | gaatgtggat  | acgcagggtga | actatggaa   | ttacatgtcc  | 780  |
| aaagtttca   | acctggacgc  | gaaatactct  | agcaccgaca  | aacaggaaac  | cctgaaagtg  | 840  |
| gcagcaaaag  | acattcaaat  | caagattgaa  | caaagattc   | aagcggagaa  | gagcacgcag  | 900  |
| tggctgcgtg  | aaactatcag  | cgccttgg    | aaaacccagc  | cgcaatggaa  | caaagaaacc  | 960  |
| gagaattaca  | gcaagggtgg  | tggtgaggac  | cacctgcaag  | gtggcgact   | gctgtatgtt  | 1020 |
| aacgcacagcc | gtaccccttg  | ggcgaatagc  | gattaccgtc  | gtctgaatcg  | caccgcaacc  | 1080 |
| aatcagacgg  | gcacgatcga  | taagtctatt  | ctggacgacg  | agtctgaccc  | aaaccacatg  | 1140 |
| ggcggttgc   | actttctgct  | ggcgaacgac  | gtcgacctga  | gcaatccgg   | cgtgcaggct  | 1200 |
| gagcagctga  | atcaaatcca  | ctatctgtat  | aattgggggtt | ccattgtat   | gggtgacaag  | 1260 |
| gatgcgaact  | ttgacggcat  | tcgtgtcgat  | gcagttgaca  | acgtggacgc  | ggacatgtt   | 1320 |
| caactgtata  | ccaattactt  | ccgtgagttac | tacgggtgt   | acaagagcga  | agctaacgca  | 1380 |
| ctggctcaca  | tcagcgttct  | ggaggcgtgg  | agcctgaaatg | ataatcatta  | caatgacaag  | 1440 |
| accgatggt   | cgccactggc  | aatggagaat  | aagcaacgtc  | tggcgcttt   | gtttcggtt   | 1500 |
| gcgaaaccga  | tcaaagagcg  | tacccggca   | gtgagccgc   | tgtataacaa  | cacccat     | 1560 |
| accacccagc  | gtgatgaaaa  | gaccgattgg  | attaacaaag  | acggtagcaa  | ggcttacaac  | 1620 |
| gaagatggca  | cggtaaaaca  | atcgaccatc  | ggtaagtaca  | acgagaata   | cggtgacgca  | 1680 |
| tccggtaact  | acgttttcat  | ccgtgcccac  | gataacaacg  | tccaggacat  | catcgccag   | 1740 |
| atcatcaaga  | aagagatcaa  | cccgaaaagc  | gacggcttca  | ccatcacca   | cgccgaaatg  | 1800 |
| aagcaaggct  | ttgaaatcta  | taacaaagat  | atgctgtcg   | gcaaaaaaa   | gtataccctg  | 1860 |
| aataacattc  | cggcagcgt   | tgccgtat    | ttgcagaata  | tggaaacgt   | tacccgcgt   | 1920 |
| tattacggtg  | atctgtatac  | ggacgacggt  | cactacatgg  | aaaccaatc   | tccgtattac  | 1980 |
| gataccatcg  | tgaatttgat  | gaagagccgt  | atcaagttat  | tttcgggtgg  | ccaggcgca   | 2040 |
| cgtagctatt  | ggctgcccac  | cgacggtaag  | atggacaata  | gcaacgttga  | gctgtaccgc  | 2100 |
| acgaatgagg  | tttacacgag  | cgtgcgtat   | ggtaaggata  | tcatgaccgc  | taatgatacc  | 2160 |
| gaaggctcta  | agtattcccg  | caccagcgcc  | caagtcac    | tggcgccgaa  | caatccgaaag | 2220 |
| ctgaatctgg  | acccaaagcgc | caagttgaat  | gtggagatgg  | gcaaaatcca  | tgcgaatcag  | 2280 |
| aagtatcg    | cactgattgt  | cggcactgc   | gacggcatta  | agaactttac  | ttccgacgc   | 2340 |
| gacgcccattg | cagcgggtt   | tgtgaaagaa  | accgatagca  | acggcggt    | gacccgtt    | 2400 |
| gctaacgaca  | ttaagggtca  | cgaaacgttt  | gatatgagcg  | gtttcggtc   | gggtgtgggt  | 2460 |
| cgggtgggt   | catctgacaa  | tcaggacatt  | cgtgtgcgc   | cgagcaccga  | ggcaaaagaaa | 2520 |
| gaaggtgagc  | tgaccttgaa  | ggcgcacggaa | gctgtatgata | gcaagctgtat | ttacgaaaggc | 2580 |
| tttagcaatt  | tccagacgt   | cccagatggc  | agcgatccgt  | ccgtgtatac  | gaaccgcaag  | 2640 |

-continued

---

|                                                                      |      |
|----------------------------------------------------------------------|------|
| attgcggaga acgtggatct gttcaaaaagc tgggggtgtca ccagcttga gatggcacccg  | 2700 |
| caattttgtct cggcggatga tggcaccttt ctggatagcg ttattcagaa tggctacgccc  | 2760 |
| ttcgcggacc gttatgaccc ggccatgtcc aagaacaaca agtatggtag caaagaggac    | 2820 |
| ctgcgtgatg cactgaaagc actgcataag gcggttattc aagctatcgc agactgggtt    | 2880 |
| ccagaccaga tctaccagct gccgggcaaa gaagttgtca ccgcaccccg tacggatgg     | 2940 |
| gtcgccgta agatcgaga cgcgattatc gaccattctc tggatgttgc aaacagcaaa      | 3000 |
| agcagcggca aagattatca agcaaagtac ggtggcgagt tccctggccga gctgaaagcc   | 3060 |
| aaataccccc aaatgttcaa agttaacatg attagcacgg gtaagecgat tggatgactcc   | 3120 |
| gtgaaaattga agcaatggaa agccgagttc ttcaatggca ccaacgtttt ggaacgtgg    | 3180 |
| gtcggctatg ttctgagcga cgaggcgacc ggttaagtattt tcacgggtgac caaagaaggc | 3240 |
| aatttcattt cgctgcaact gacgggtaaa gagaaagtta tcacgggtttt ctccagcgat   | 3300 |
| ggtaagggta tcaccttattt cggtacgagc ggtacgcagg cgaagtctgc gtttggtaacc  | 3360 |
| ttcaatggta acacctacta tttcgacgcg cgtggccaca tgggttaccaa tagcgaatac   | 3420 |
| agccccaaatg gcaaggacgt ctaccgtttt ctgcccgaacg gtatcatgct gagcaatgcg  | 3480 |
| ttttacattt atgcgaacgg taatacctac ctgtacaact ctaagggtca aatgtacaaa    | 3540 |
| ggcgggttaca cgaaattcga tggttctgaa acggataagg acggtaaaga gtccaaaggc   | 3600 |
| gtcaagttcc gctactttac gaacgaaggc gtcatggccca agggtgttac cgtcattgtat  | 3660 |
| ggttttaccc aatacttgg tgaggacggc tttcaaggca aggataagct ggtcaccc       | 3720 |
| aagggaaga cgtattactt cgacgcacac actggtaatg gtatcaaaga tacctggcgc     | 3780 |
| aatatcaatg gtaaaatggta ctatttcgac gcgaatggcg ttgctgcgc cggtgccag     | 3840 |
| gtgattaacg gccagaaact gtacttcaac gaggatggct cccaaagtcaa aggccgcgt    | 3900 |
| gttaagaacg cagacggcac ctatagcaaa tacaagaag gttttggta gctggttact      | 3960 |
| aacgagtttt tcacgactga tggcaatgtt tggtaactacg ccgggtgcaaa tggtaaaacc  | 4020 |
| gttaccggtg cacaagtgtat caacggccaa cattttgtact tcaatgcggc cggttccag   | 4080 |
| gtgaagggtg gcgttgcataa gaacgcggat ggcacccata gcaagtacaa tgcttagcact  | 4140 |
| ggtaaacgtc tgacgaacga gttttttacg accggtgata acaattggta ttacattggc    | 4200 |
| gcaaaacggta agagcgtgac ggggtgaggc aagattgggt atgataactt ctttttcgc    | 4260 |
| aaggatggca aacaagttaa aggtcaaaacc gtcagcgcgc gtaatggtc cattagctac    | 4320 |
| tactacggtg acagcggcaa gcgtgcgggtt agcacctggta ttgagattca gcccgggtt   | 4380 |
| tatgtgtatt tcgacaaaaa cggtttggcg taccctccgc gtgttctgaa ttaa          | 4434 |

&lt;210&gt; SEQ ID NO 2

&lt;211&gt; LENGTH: 8455

&lt;212&gt; TYPE: DNA

&lt;213&gt; ORGANISM: artificial sequence

&lt;220&gt; FEATURE:

&lt;223&gt; OTHER INFORMATION: plasmid pMP52

&lt;400&gt; SEQUENCE: 2

|                                                                      |     |
|----------------------------------------------------------------------|-----|
| ctcatgacca aaatccctta acgtgagttt cgcgcgcgtc gttccactga gcgtcagacc    | 60  |
| ccgttagaaaa gatcaaagga tcttcttgcg atccctttttt tctgcgcgtt atctgtgtct  | 120 |
| tgcaaaacaaa aaaaccaccc ctaccagcgg tgggttgcgtt gcccggatcaa gagctaccaa | 180 |
| ctctttttcc gaaggtaact ggcttcagca gagcgcagat accaaatact gttctctag     | 240 |
| tgttagccgta gttagcccac cacttcaaga actctgttagc accgcctaca tacctcgctc  | 300 |

-continued

---

|                                                                     |      |
|---------------------------------------------------------------------|------|
| tgctaatcct gttaccagtg gctgctgcca gtggcgataa gtcgtgtctt accgggttgg   | 360  |
| actcaagacg atagttaccg gataaggcgc agcggtcggg ctgaacgggg ggttctgtca   | 420  |
| cacageccag cttggagcga acgacctaca cggaaactgag atacctacag cgtgagctat  | 480  |
| gagaaagcgc cacgttccc gaagggagaa aggccgacag gtatccggta agccgcagg     | 540  |
| tcggaacagg agagcgcacg agggagctc cagggggaaa cgcctggat ctttatagtc     | 600  |
| ctgtcggtt tcgcccaccc tgacttgacg gtcgatttt gtgtatgtcg tcagggggc      | 660  |
| ggagcctatg gaaaaacgcc agcaacgcgg ccttttacg gttcctggcc ttttgcggc     | 720  |
| cttttgtca catgttctt cctgcgttat cccctgattc tggataac cgtattaccg       | 780  |
| cctttgagtg agctgatacc gtcgcccga gccgaacgac cgagcgcacg gagtcagtga    | 840  |
| gcgaggaagc ggaaggcgcag agtagggaaac tgccaggcat caaactaagc agaaggcccc | 900  |
| tgacggatgg ctttttgcg tttctacaaa ctctttctgt gttgtaaaac gacggccagt    | 960  |
| cttaagctcg ggccccctgg gcggttctga taacgagtaa tcgttaatcc gcaaataacg   | 1020 |
| taaaaaaccgc cttcggcggg tttttttagt gggggagttt agggaaagag catttgcag   | 1080 |
| aatatattaag ggccctgtc actttgcttg atatatgaga attatattaac cttataaatg  | 1140 |
| agaaaaaaagc aacgcacttt aaataagata cggtgcttt tcgattgtat aacacctata   | 1200 |
| attaaactat tcatctatta tttatgattt tttgtatata caatatttct agtttgtaa    | 1260 |
| agagaattaa gaaaataaaat ctcgaaaata ataaaggaa aatcagttt tgatataaaa    | 1320 |
| attatacatg tcaacgataa tacaaaatata aataacaaact ataagatgtt atcagtattt | 1380 |
| attatgcatt tagaataaaat tttgtgtcgc ccttaattgt gagcggataa caattacgag  | 1440 |
| cttcatgcac agtgaatca tgaaaaattt atttgcttt tgagcggata acaattataa     | 1500 |
| tatgtggat tggagcgct cacaattcca caacggtttc cctctagaaa taattttgtt     | 1560 |
| taactttga attctctaga ggaaggtaaa acatatggac gaaacgcagg ataagaccgt    | 1620 |
| gacgcagagc aacagcggca ccaccgcctc cctggtaact agccctgaag ccacgaaaga   | 1680 |
| ggcggacaaa cgcacgaaca ctaaagagc cgacgttctg acgcctgcaaa aagaaacgaa   | 1740 |
| cgcagtcgag actgcgcacca ccactaacac ccaggcgcacg gggaggccg ccacgaccgc  | 1800 |
| gaccaccgcg gacgtcgcgg tggctgcggt gccgaacaaa gaagcggtcg ttaccacgga   | 1860 |
| tgcgtccggcg gtcacgaccg agaaagcggaa agaacagccg gtcaccgtta aagcagaagt | 1920 |
| cgtcaatacg gaagtgaaag cgccggaaagc ggctctgaaa gacagcggagg ttgaggcagc | 1980 |
| gctgagcctg aagaacatca agaacattga tggcaagtt tactatgtt atgaggatgg     | 2040 |
| cagccacaaa gagaatttcg ctattaccgt gaatggccag ctgctgtact ttggtaaaga   | 2100 |
| cggtgtcgctg acgtcctcta gcacgttattc ttttacccca ggcactacca atatcgtgga | 2160 |
| cggtttttagc attaacaacc gcgttacga cagcagcgcag ggcgttgcg agctgtatcg   | 2220 |
| cggttacttg accgcgcacca gctggatctcg tccggctacg atcatcaaaat atgggttac | 2280 |
| gtggcaagcg tccaccgcgg aggatttcg tccgctgtg atggcatggt ggccgaatgt     | 2340 |
| ggatacgcacg gtgaacttatt tgaattacat gtccaaaggt ttcaacctgg acgcgaaata | 2400 |
| ctctagcacc gacaaacagg aaaccctgaa agtggcgcacca aaagacatcc aatcaagat  | 2460 |
| tgaacaaaag attcaagcgg agaagagcac gcagtggctg cgtgaaacta tcagcgcctt   | 2520 |
| tgtgaaaacc cagccgcagt ggaacaaaga aaccgagaat tacagcaagg gtgggtggta   | 2580 |
| ggaccacctg caagggtggcg cactgctgta tggtaacgac agccgtaccc cttggcgaa   | 2640 |
| tagcgattac cgtcgctctga atcgcaccgc aaccaatcag acgggcacga tcgataagtc  | 2700 |

-continued

---

|                                 |                      |                       |      |
|---------------------------------|----------------------|-----------------------|------|
| tattctggac gagcagtctg acccaaacc | catggcggt ttcgacttgc | tgctggcgaa            | 2760 |
| cgacgtcgac ctgagcaatc           | cggtcgta ggctgagcag  | ctgaatcaaa tccactatct | 2820 |
| gatgaattgg ggttccattg           | tgtatgggtga          | caaggatgcg aactttgacg | 2880 |
| cgatgcagtt gacaacgtgg           | acgcccacat           | gttgcactgtataccatt    | 2940 |
| gtactacggt gtgaacaaga           | gchgagctaa           | cgcaactggc            | 3000 |
| gtggagcctg aatgataatc           | attacaatga           | caagacccat            | 3060 |
| gaataagcaa cgtctggcgc           | tgttggtttc           | gttggcgaaa            | 3120 |
| ggcagtgagc cccgtgtata           | acaacaccc            | caataccacc            | 3180 |
| ttggattaac aaagacggta           | gcaaggctta           | caacgaagat            | 3240 |
| catcggtaa                       | gataacccg            | cgatccggtaactacgttt   | 3300 |
| ccacgataac aacgtccagg           | acatcategc           | cgagatcatc            | 3360 |
| aagcgcggc ttcaccatca            | ccgacgcccga          | aatgaagcaa            | 3420 |
| agatatgctg tcgagcgaca           | aaaagtatac           | cctgaataac            | 3480 |
| gatgttgcg aatatggaaa            | cgattacccg           | cgtctattac            | 3540 |
| cggtcactac atggaaacca           | aatctccgtat          | ttacgataacc           | 3600 |
| ccgttatcaag tatgttccgg          | gtggccaggc           | gcaacgtacg            | 3660 |
| taagatggac aatagcgacg           | tttagtctgtat         | ccgcacgaat            | 3720 |
| ctatggtaag gatatcatga           | ccgctaataatga        | taccgaaggc            | 3780 |
| cggccaagtc accttggcgc           | cgaacaatcc           | gaagctgaat            | 3840 |
| gaatgtggag atggggcaaaa          | tccatgcgaa           | tcagaagtat            | 3900 |
| tgccggacggc attaagaact          | ttacttccga           | cgccggacgc            | 3960 |
| agaaaccat agcaacggcg            | tgctgacctt           | cggtgctaac            | 4020 |
| gtttgatatg agcggtttcg           | ttggcggtgt           | ggttccgggt            | 4080 |
| cattcgtgtt ggcggcagca           | ccgaggcaaa           | gaaagaaggt            | 4140 |
| ggaagcgtat gatagccagc           | tgatttacga           | aggctttacg            | 4200 |
| tggcagcgtat cgtccgtgt           | atacgaaccc           | caagattgcg            | 4260 |
| aagctgggggt gtcaccagct          | tttagatggc           | accgcaattt            | 4320 |
| ctttctggat agcggttattc          | agaatggcta           | cgccttcgccc           | 4380 |
| gtccaagaac aacaagtatg           | gtagcaaaga           | ggacactgcgt           | 4440 |
| taaggcgggt attcaagcta           | tcgcagactg           | ggttccagac            | 4500 |
| caaagaagtt gtcaccgcca           | cccgtaacgg           | tggtgctggc            | 4560 |
| tatcgaccat tctctgtatg           | ttgcaaacag           | caaaagcagc            | 4620 |
| gtacgggtggc gagttccctgg         | ccgagctgaa           | agccaaatac            | 4680 |
| catgatttgc acgggttaagc          | cgattgtatg           | ctccgtgaaa            | 4740 |
| gtacttcaat ggcaccaacg           | tttttggaaacg         | tggtgtcggt            | 4800 |
| gaccggtaag tatttcacgg           | tgaccaaaga           | aggcaatttc            | 4860 |
| taaagagaaa gttatcacgg           | gttttccag            | cgatggtaag            | 4920 |
| gagccgtacg cagggaaatgt          | ctgctttgt            | taccttcaat            | 4980 |
| cgccgcgtggc cacatggta           | ccaaatgcga           | atacagcccg            | 5040 |
| ttttctggccg aacggtatca          | tgctgagcaa           | tgcgttttac            | 5100 |

-continued

---

|                                                                        |      |
|------------------------------------------------------------------------|------|
| ctacctgtac aactctaagg gtc当地atgtc caaaggcggt tacacgaaat tcgatgttc       | 5160 |
| tgaaacggat aaggacggta aagagtccaa ggtcgtaa ttccgctact ttacgaaacga       | 5220 |
| aggcgtcatg gccaagggtg ttaccgtcat tgatggttt acccaatact tcggtgagga       | 5280 |
| cggttcaa gcgaaggata agctggtcac cttcaaggcc aagacgtatt acttcgacgc        | 5340 |
| acacactggt aatggtatca aagatacctg ggc当地atgtc aatggtaat ggtactattt       | 5400 |
| cgacggeaat ggc当地tgcg cggccgtgc gcaggtgatt aacggccaga aactgtactt        | 5460 |
| caacgaggat ggctccaaag tcaaaggccg cgtggtaag aacgcagacg gcacctata        | 5520 |
| caaatacaaa gaaggtttt gtc当地tgcg tactaacgag ttttcacga ctgatggca          | 5580 |
| tgttggtaac tacgcccgtg caaatggtaa aaccgttacc ggtgcacaag tgatcaacgg      | 5640 |
| ccaacatggt tacttaatgc cggacgggtc ccaggtgaag ggtggcgtg tcaagaacgc       | 5700 |
| ggatggcacc tacagcaagt acaatgttag cactggtaa cgtctgacga acgagtttt        | 5760 |
| tacgaccggt gataacaatt ggtattacat tggcgcaaac ggtaagagcg tgacgggtga      | 5820 |
| ggtcaagatt ggtgatgata cttactttt cgc当地aggat ggcaaaacaag tt当地aggta       | 5880 |
| aaccgtcage gccc当地atgc gtc当地tgcg ctactactac ggtgacagcg gcaaggcgtgc      | 5940 |
| ggtagcacc tggattgaga tt当地ccggg tggatgtg tatttcgaca aaaacggttt          | 6000 |
| ggcgtaccct cccgtgttc tgaatatacg agtcttagact gcagggtacc aagctcccc       | 6060 |
| aaggcgaca ccccaataatt agccccggcg aaaggccccag tcttcgact gagccttcg       | 6120 |
| ttttatttga tgc当地ggcag ttccctactc tc当地atgggg agtccccaca ctaccatcg       | 6180 |
| cgctacggcg tt当地acttct gagttcggca tggggcagg tgggaccacc gcgctactgc       | 6240 |
| cggccaggcaa acaaggggtg tt当地gagcca tattcaggta taaatggct cgc当地atgc       | 6300 |
| ttc当地atgtt gttatggt tgtaacactg acccctattt gtttattttt ct当地atcat         | 6360 |
| tcaaatatgt atccgtcatc gagacaataa cc当地tgcataa tgcttcaata atattgaaaa     | 6420 |
| aggaagaata tgtagtattca acatttccgt gtc当地cccta ttccctttt tgccggattt      | 6480 |
| tgc当地tctg ttttgc当地 cccagaaacg ctggtaaaag taaaagatgc tgaagatcg          | 6540 |
| ttggggc当地 gagttgggtt当地 catgaaactg gatctcaaca gggtaagat cctttagat       | 6600 |
| tttccccc当地 aagaacgtt当地 tccatgtatc agcactttt aagttctgt atgtggcgc        | 6660 |
| gtattatccc gtattgacgc cggccagag caactcggtc gccc当地atca ctattctcag       | 6720 |
| aatgacttgg tt当地gactc accagtcaca gaaaagcatc ttacggatgg catgacagta       | 6780 |
| agagaattat gcaatgtgc cataaccatc agtgc当地aca ctgc当地ccaa cttacttctg       | 6840 |
| acaacgatcg gaggaccgaa ggagctacc gcttttgc acaacatggg ggatcatgt          | 6900 |
| actcgccctt当地 atcgatgggaa accggagctg aatgaaaccatc taccaaacgc cgagcgtgc  | 6960 |
| accacgatgc ctgatgc当地 ggcaacaacg ttgc当地caac tattactgg cgaactactt        | 7020 |
| actctatgtt cccggcaaca attatagac tggatggagg cggat当地atg tgc当地gg          | 7080 |
| cttctgatc cggcccttcc ggctggctgg tttattgtg ataaatccgg agccggatg         | 7140 |
| cgtggatctc cggatctatc cgc当地cgctg gggccatgc gtaaggccctc cc当地atcgta      | 7200 |
| gttatctaca cgacggggag tc当地ggact atggatgaaac gaaatagaca gatcgatgt       | 7260 |
| atagggtcct cactgattaa gcatggtaa gccc当地ccgc atc当地atggc gcaaaaccc        | 7320 |
| tc当地ggatgc gcatgatgc gccc当地aga gactcaatc agggtggtaa atatgaaacc         | 7380 |
| agtaacgtt当地 tacgatgtcg cagatgtgc cggatctct tatcagacccg tt当地ccgcgt      | 7440 |
| ggatgaaaccag gccc当地ccacg tt当地tgc当地aa aacgc当地ggaa aaagtggaa cggc当地atggc | 7500 |

-continued

---

```

ggagctgaat tacattccca accgcgtggc acaacaactg gggggcaac agtcgttgct 7560
gattggcggtt gccaccccca gtcgtggccct gcacgcgcggc tcgcaaattg tcgcggcgat 7620
taaatctcgc gccgatcaac tgggtgccag cgtgggtggtg tcgatggtag aacgaagcg 7680
cgtcgaagcc tgtaaaagcg 17740
cggtgcacaa tcttctcgcg caacgcgtca gtgggctgat 7740
cattaaactat ccgcgtggatg accaggatgc cattgctgtg gaagctgcct gcactaatgt 7800
tccggcggtt tttcttgatg tctctgacca gacacccatc aacagtattt ttttctccca 7860
tgaggacggt acgcgactgg gcgtggagca tctggtcgca ttgggtcacc agcaaatcg 7920
gctgttagcg ggccattaa gttctgtctc ggccgcgtctg cgtctggctg gctggcataa 7980
atatctcaact cgcaatcaaa ttcaagccat agcggaaacgg gaaggcgact ggagtgcac 8040
gtcccggtttt caacaaacca tgcaaatgtt gaatgaggggc atcgatccca ctgcgtatgt 8100
ggttgccaac gatcagatgg cgctggcgcc aatgcgcgcattaccgagt ccgggctgcg 8160
cgttggtgcg gatatctcg tagtggata cgacgatacc gaagatagtt catgttatat 8220
cccgccgttta accaccatca aacaggattt tcgcctgtctg gggcaaaacca gcgtggacccg 8280
cttgctgcaa ctctctcagg gccaggcggtt gaagggaat cagctgttc cagtcact 8340
ggtgaaaaga aaaaccaccc tggcgcccaa tacgcaaaacc gcctctcccc gcgcgttggc 8400
cgattcatta atgcagctgg cacgacaggt ttcccgactg gaaagcgggc agtga 8455

```

&lt;210&gt; SEQ ID NO 3

&lt;211&gt; LENGTH: 1518

&lt;212&gt; TYPE: PRT

<213> ORGANISM: *Streptococcus salivarius*

&lt;400&gt; SEQUENCE: 3

```

Met Glu Asn Lys Ile His Tyr Lys Leu His Lys Val Lys Lys Gln Trp
1 5 10 15

```

```

Val Thr Ile Ala Val Ala Ser Val Ala Leu Ala Thr Val Leu Gly Gly
20 25 30

```

```

Leu Ser Val Thr Thr Ser Ser Val Ser Ala Asp Glu Thr Gln Asp Lys
35 40 45

```

```

Thr Val Thr Gln Ser Asn Ser Gly Thr Thr Ala Ser Leu Val Thr Ser
50 55 60

```

```

Pro Glu Ala Thr Lys Glu Ala Asp Lys Arg Thr Asn Thr Lys Glu Ala
65 70 75 80

```

```

Asp Val Leu Thr Pro Ala Lys Glu Thr Asn Ala Val Glu Thr Ala Thr
85 90 95

```

```

Thr Thr Asn Thr Gln Ala Thr Ala Glu Ala Ala Thr Thr Ala Thr Thr
100 105 110

```

```

Ala Asp Val Ala Val Ala Ala Val Pro Asn Lys Glu Ala Val Val Thr
115 120 125

```

```

Thr Asp Ala Pro Ala Val Thr Thr Glu Lys Ala Glu Glu Gln Pro Ala
130 135 140

```

```

Thr Val Lys Ala Glu Val Val Asn Thr Glu Val Lys Ala Pro Glu Ala
145 150 155 160

```

```

Ala Leu Lys Asp Ser Glu Val Glu Ala Ala Leu Ser Leu Lys Asn Ile
165 170 175

```

```

Lys Asn Ile Asp Gly Lys Tyr Tyr Val Asn Glu Asp Gly Ser His
180 185 190

```

```

Lys Glu Asn Phe Ala Ile Thr Val Asn Gly Gln Leu Leu Tyr Phe Gly
195 200 205

```

-continued

---

Lys Asp Gly Ala Leu Thr Ser Ser Ser Thr Tyr Ser Phe Thr Pro Gly  
 210 215 220

Thr Thr Asn Ile Val Asp Gly Phe Ser Ile Asn Asn Arg Ala Tyr Asp  
 225 230 235 240

Ser Ser Glu Ala Ser Phe Glu Leu Ile Asp Gly Tyr Leu Thr Ala Asp  
 245 250 255

Ser Trp Tyr Arg Pro Ala Ser Ile Ile Lys Asp Gly Val Thr Trp Gln  
 260 265 270

Ala Ser Thr Ala Glu Asp Phe Arg Pro Leu Leu Met Ala Trp Trp Pro  
 275 280 285

Asn Val Asp Thr Gln Val Asn Tyr Leu Asn Tyr Met Ser Lys Val Phe  
 290 295 300

Asn Leu Asp Ala Lys Tyr Ser Ser Thr Asp Lys Gln Glu Thr Leu Lys  
 305 310 315 320

Val Ala Ala Lys Asp Ile Gln Ile Lys Ile Glu Gln Lys Ile Gln Ala  
 325 330 335

Glu Lys Ser Thr Gln Trp Leu Arg Glu Thr Ile Ser Ala Phe Val Lys  
 340 345 350

Thr Gln Pro Gln Trp Asn Lys Glu Thr Glu Asn Tyr Ser Lys Gly Gly  
 355 360 365

Gly Glu Asp His Leu Gln Gly Ala Leu Leu Tyr Val Asn Asp Ser  
 370 375 380

Arg Thr Pro Trp Ala Asn Ser Asp Tyr Arg Arg Leu Asn Arg Thr Ala  
 385 390 395 400

Thr Asn Gln Thr Gly Thr Ile Asp Lys Ser Ile Leu Asp Glu Gln Ser  
 405 410 415

Asp Pro Asn His Met Gly Gly Phe Asp Phe Leu Leu Ala Asn Asp Val  
 420 425 430

Asp Leu Ser Asn Pro Val Val Gln Ala Glu Gln Leu Asn Gln Ile His  
 435 440 445

Tyr Leu Met Asn Trp Gly Ser Ile Val Met Gly Asp Lys Asp Ala Asn  
 450 455 460

Phe Asp Gly Ile Arg Val Asp Ala Val Asp Asn Val Asp Ala Asp Met  
 465 470 475 480

Leu Gln Leu Tyr Thr Asn Tyr Phe Arg Glu Tyr Tyr Gly Val Asn Lys  
 485 490 495

Ser Glu Ala Asn Ala Leu Ala His Ile Ser Val Leu Glu Ala Trp Ser  
 500 505 510

Leu Asn Asp Asn His Tyr Asn Asp Lys Thr Asp Gly Ala Ala Leu Ala  
 515 520 525

Met Glu Asn Lys Gln Arg Leu Ala Leu Phe Ser Leu Ala Lys Pro  
 530 535 540

Ile Lys Glu Arg Thr Pro Ala Val Ser Pro Leu Tyr Asn Asn Thr Phe  
 545 550 555 560

Asn Thr Thr Gln Arg Asp Glu Lys Thr Asp Trp Ile Asn Lys Asp Gly  
 565 570 575

Ser Lys Ala Tyr Asn Glu Asp Gly Thr Val Lys Gln Ser Thr Ile Gly  
 580 585 590

Lys Tyr Asn Glu Lys Tyr Gly Asp Ala Ser Gly Asn Tyr Val Phe Ile  
 595 600 605

Arg Ala His Asp Asn Asn Val Gln Asp Ile Ile Ala Glu Ile Ile Lys  
 610 615 620

## US 9,096,956 B2

27

28

-continued

---

Lys Glu Ile Asn Pro Lys Ser Asp Gly Phe Thr Ile Thr Asp Ala Glu  
 625 630 635 640

Met Lys Gln Ala Phe Glu Ile Tyr Asn Lys Asp Met Leu Ser Ser Asp  
 645 650 655

Lys Lys Tyr Thr Leu Asn Asn Ile Pro Ala Ala Tyr Ala Val Met Leu  
 660 665 670

Gln Asn Met Glu Thr Ile Thr Arg Val Tyr Tyr Gly Asp Leu Tyr Thr  
 675 680 685

Asp Asp Gly His Tyr Met Glu Thr Lys Ser Pro Tyr Tyr Asp Thr Ile  
 690 695 700

Val Asn Leu Met Lys Ser Arg Ile Lys Tyr Val Ser Gly Gly Gln Ala  
 705 710 715 720

Gln Arg Ser Tyr Trp Leu Pro Thr Asp Gly Lys Met Asp Asn Ser Asp  
 725 730 735

Val Glu Leu Tyr Arg Thr Asn Glu Val Tyr Thr Ser Val Arg Tyr Gly  
 740 745 750

Lys Asp Ile Met Thr Ala Asn Asp Thr Glu Gly Ser Lys Tyr Ser Arg  
 755 760 765

Thr Ser Gly Gln Val Thr Leu Val Ala Asn Asn Pro Lys Leu Asn Leu  
 770 775 780

Asp Gln Ser Ala Lys Leu Asn Val Glu Met Gly Lys Ile His Ala Asn  
 785 790 795 800

Gln Lys Tyr Arg Ala Leu Ile Val Gly Thr Ala Asp Gly Ile Lys Asn  
 805 810 815

Phe Thr Ser Asp Ala Asp Ala Ile Ala Ala Gly Tyr Val Lys Glu Thr  
 820 825 830

Asp Ser Asn Gly Val Leu Thr Phe Gly Ala Asn Asp Ile Lys Gly Tyr  
 835 840 845

Glu Thr Phe Asp Met Ser Gly Phe Val Ala Val Trp Val Pro Val Gly  
 850 855 860

Ala Ser Asp Asn Gln Asp Ile Arg Val Ala Pro Ser Thr Glu Ala Lys  
 865 870 875 880

Lys Glu Gly Glu Leu Thr Leu Lys Ala Thr Glu Ala Tyr Asp Ser Gln  
 885 890 895

Leu Ile Tyr Glu Gly Phe Ser Asn Phe Gln Thr Ile Pro Asp Gly Ser  
 900 905 910

Asp Pro Ser Val Tyr Thr Asn Arg Lys Ile Ala Glu Asn Val Asp Leu  
 915 920 925

Phe Lys Ser Trp Gly Val Thr Ser Phe Glu Met Ala Pro Gln Phe Val  
 930 935 940

Ser Ala Asp Asp Gly Thr Phe Leu Asp Ser Val Ile Gln Asn Gly Tyr  
 945 950 955 960

Ala Phe Ala Asp Arg Tyr Asp Leu Ala Met Ser Lys Asn Asn Lys Tyr  
 965 970 975

Gly Ser Lys Glu Asp Leu Arg Asp Ala Leu Lys Ala Leu His Lys Ala  
 980 985 990

Gly Ile Gln Ala Ile Ala Asp Trp Val Pro Asp Gln Ile Tyr Gln Leu  
 995 1000 1005

Pro Gly Lys Glu Val Val Thr Ala Thr Arg Thr Asp Gly Ala Gly  
 1010 1015 1020

Arg Lys Ile Ala Asp Ala Ile Ile Asp His Ser Leu Tyr Val Ala  
 1025 1030 1035

-continued

---

Asn Ser Lys Ser Ser Gly Lys Asp Tyr Gln Ala Lys Tyr Gly Gly  
 1040 1045 1050  
 Glu Phe Leu Ala Glu Leu Lys Ala Lys Tyr Pro Glu Met Phe Lys  
 1055 1060 1065  
 Val Asn Met Ile Ser Thr Gly Lys Pro Ile Asp Asp Ser Val Lys  
 1070 1075 1080  
 Leu Lys Gln Trp Lys Ala Glu Tyr Phe Asn Gly Thr Asn Val Leu  
 1085 1090 1095  
 Glu Arg Gly Val Gly Tyr Val Leu Ser Asp Glu Ala Thr Gly Lys  
 1100 1105 1110  
 Tyr Phe Thr Val Thr Lys Glu Gly Asn Phe Ile Pro Leu Gln Leu  
 1115 1120 1125  
 Thr Gly Lys Glu Lys Val Ile Thr Gly Phe Ser Ser Asp Gly Lys  
 1130 1135 1140  
 Gly Ile Thr Tyr Phe Gly Thr Ser Gly Thr Gln Ala Lys Ser Ala  
 1145 1150 1155  
 Phe Val Thr Phe Asn Gly Asn Thr Tyr Tyr Phe Asp Ala Arg Gly  
 1160 1165 1170  
 His Met Val Thr Asn Ser Glu Tyr Ser Pro Asn Gly Lys Asp Val  
 1175 1180 1185  
 Tyr Arg Phe Leu Pro Asn Gly Ile Met Leu Ser Asn Ala Phe Tyr  
 1190 1195 1200  
 Ile Asp Ala Asn Gly Asn Thr Tyr Leu Tyr Asn Ser Lys Gly Gln  
 1205 1210 1215  
 Met Tyr Lys Gly Gly Tyr Thr Lys Phe Asp Val Ser Glu Thr Asp  
 1220 1225 1230  
 Lys Asp Gly Lys Glu Ser Lys Val Val Lys Phe Arg Tyr Phe Thr  
 1235 1240 1245  
 Asn Glu Gly Val Met Ala Lys Gly Val Thr Val Ile Asp Gly Phe  
 1250 1255 1260  
 Thr Gln Tyr Phe Gly Glu Asp Gly Phe Gln Ala Lys Asp Lys Leu  
 1265 1270 1275  
 Val Thr Phe Lys Gly Lys Thr Tyr Tyr Phe Asp Ala His Thr Gly  
 1280 1285 1290  
 Asn Gly Ile Lys Asp Thr Trp Arg Asn Ile Asn Gly Lys Trp Tyr  
 1295 1300 1305  
 Tyr Phe Asp Ala Asn Gly Val Ala Ala Thr Gly Ala Gln Val Ile  
 1310 1315 1320  
 Asn Gly Gln Lys Leu Tyr Phe Asn Glu Asp Gly Ser Gln Val Lys  
 1325 1330 1335  
 Gly Gly Val Val Lys Asn Ala Asp Gly Thr Tyr Ser Lys Tyr Lys  
 1340 1345 1350  
 Glu Gly Phe Gly Glu Leu Val Thr Asn Glu Phe Phe Thr Thr Asp  
 1355 1360 1365  
 Gly Asn Val Trp Tyr Tyr Ala Gly Ala Asn Gly Lys Thr Val Thr  
 1370 1375 1380  
 Gly Ala Gln Val Ile Asn Gly Gln His Leu Tyr Phe Asn Ala Asp  
 1385 1390 1395  
 Gly Ser Gln Val Lys Gly Gly Val Val Lys Asn Ala Asp Gly Thr  
 1400 1405 1410  
 Tyr Ser Lys Tyr Asn Ala Ser Thr Gly Glu Arg Leu Thr Asn Glu  
 1415 1420 1425

-continued

---

|      |     |     |     |     |     |     |     |     |     |     |     |      |     |     |
|------|-----|-----|-----|-----|-----|-----|-----|-----|-----|-----|-----|------|-----|-----|
| Phe  | Phe | Thr | Thr | Gly | Asp | Asn | Asn | Trp | Tyr | Tyr | Ile | Gly  | Ala | Asn |
| 1430 |     |     |     |     |     |     |     |     |     |     |     |      |     |     |
|      |     |     |     |     |     |     |     |     |     |     |     | 1440 |     |     |
| Gly  | Lys | Ser | Val | Thr | Gly | Glu | Val | Lys | Ile | Gly | Asp | Asp  | Thr | Tyr |
| 1445 |     |     |     |     |     |     |     |     |     |     |     |      |     |     |
|      |     |     |     |     |     |     |     |     |     |     |     | 1455 |     |     |
| Phe  | Phe | Ala | Lys | Asp | Gly | Lys | Gln | Val | Lys | Gly | Gln | Thr  | Val | Ser |
| 1460 |     |     |     |     |     |     |     |     |     |     |     |      |     |     |
|      |     |     |     |     |     |     |     |     |     |     |     | 1470 |     |     |
| Ala  | Gly | Asn | Gly | Arg | Ile | Ser | Tyr | Tyr | Tyr | Gly | Asp | Ser  | Gly | Lys |
| 1475 |     |     |     |     |     |     |     |     |     |     |     |      |     |     |
|      |     |     |     |     |     |     |     |     |     |     |     | 1485 |     |     |
| Arg  | Ala | Val | Ser | Thr | Trp | Ile | Glu | Ile | Gln | Pro | Gly | Val  | Tyr | Val |
| 1490 |     |     |     |     |     |     |     |     |     |     |     |      |     |     |
|      |     |     |     |     |     |     |     |     |     |     |     | 1500 |     |     |
| Tyr  | Phe | Asp | Lys | Asn | Gly | Leu | Ala | Tyr | Pro | Pro | Arg | Val  | Leu | Asn |
| 1505 |     |     |     |     |     |     |     |     |     |     |     |      |     |     |
|      |     |     |     |     |     |     |     |     |     |     |     | 1515 |     |     |

---

What is claimed is:

1. A process comprising  
subjecting one or more filaments comprising poly( $\alpha$ (1 $\rightarrow$ 3)  
glucan) to a tension below the breaking strength of the  
one or more filaments at 350° C.;  
subjecting the thus tensioned one or more filaments to a  
first thermal exposure by heating said one or more filaments  
to a temperature in the range of 160 to 200° C. in  
air for a duration in the range of 5 to 15 minutes;  
subjecting the thus heated one or more filaments to a sec-  
ond thermal exposure by further heating said one or  
more filaments, still under tension, from a first tempera-  
ture in the range of 200 to 250° C. to a second tempera-  
ture in the range of 300 to 350° C., thereby preparing one  
or more thermally stabilized filaments;  
subjecting said one or more stabilized filaments in a zero  
tension state to a third thermal exposure by heating said  
one or stabilized filaments to a temperature in the range  
20
2. The process of claim 1 wherein the first thermal exposure  
is effected at a temperature in the range of 175 to 185° C. for  
a duration of 7.5 to 12.5 minutes.
3. The process of claim 1 wherein said second thermal  
exposure is effected in a series of well-defined steps between  
the first temperature and the second temperature, with a hold  
period between steps, and a heating rate from step to step in  
excess of 10° C. per minute.
4. The process of claim 1 wherein said first temperature is  
in the range of 230-250° C., and said second temperature is in  
the range of 310 to 330° C.
5. The process of claim 1 wherein the third thermal expo-  
sure is effected at a temperature in the range of 800 to 1000°  
C. for a duration in the range of 1 to 2 minutes.

\* \* \* \* \*